

# UNITED STATES PATENT OFFICE.

FRANK T. COOK, OF ANTELOPE, OREGON.

## LUBRICANT.

SPECIFICATION forming part of Letters Patent No. 635,308, dated October 24, 1899.

Application filed January 20, 1898. Serial No. 667,324. (No specimens.)

*To all whom it may concern:*

Be it known that I, FRANK T. COOK, residing at Antelope, in the county of Wasco and State of Oregon, have invented a new and useful Chain-Lubricant, of which the following is a specification.

This invention relates to compositions for lubricants, and particularly to lubricants to be used upon bicycle and other chains.

10 The object is to provide a lubricant composed of a minimum number of ingredients and which is cheap in production, the same containing no oil to collect dirt and dust and soil the clothes of the rider and also being 15 more lasting and effective than the lubricants now in general use.

In the manufacture of my improved composition I first take about one pound of beeswax and dissolve the same by heat, adding 20 thereto one-half pound of the best plumbago, stirring the same well, and permitting the resulting mixture to cool to about 90° Fahrenheit. I then add one and one-half ounces of the best glycerin, mixing the same thoroughly 25 with the beeswax and plumbago. The mixture is then poured into molds of suitable form and permitted to cool.

The glycerin is used for the purpose of keeping the mixture from becoming too hard when the same has become cool, and only a 30 sufficient quantity of the glycerin to effect the desired result is used. Other ingredients might be used to serve the same function as the glycerin—as, for instance, sperm-oil.

A chain-lubricant composed of the ingredients above set forth and in approximately the quantities specified is very effective in operation, cheap in production, and possesses the advantage of not gumming or collecting 35 dirt and dust, as is the case with lubricants 40 containing a large percentage of oil, so that the clothing of the rider is not soiled thereby.

Having thus fully described my composition, what I claim as new, and desire to secure by Letters Patent of the United States, is— 45

A lubricant composed of beeswax and plumbago, and a sufficient quantity of glycerin to prevent the lubricant from becoming too hard, substantially as set forth.

FRANK T. COOK.

Witnesses:

ANTONE NELSON,  
W. E. KEMP.